

Feb. 13, 1940.

W. HICKOK

2,189,986

METHOD OF MAKING MOSAIC ELECTRODES

Filed March 26, 1938

*Fig. 1*



*Fig. 2*



*Fig. 3*



INVENTOR.  
WILLARD HICKOK

BY

*Charles McLean*  
ATTORNEY.

## UNITED STATES PATENT OFFICE

2,189,986

## METHOD OF MAKING MOSAIC ELECTRODES

Willard Hickok, Bloomfield, N. J., assignor, by  
mesne assignments, to Radio Corporation of  
America, New York, N. Y., a corporation of  
Delaware

Application March 26, 1938, Serial No. 198,209

2 Claims. (Cl. 250—27.5)

My invention relates to improvements in cathode ray television tubes and particularly to improved methods of manufacturing television tubes which have photosensitive mosaic electrodes.

It has been found that in cathode ray tubes with a conventional mosaic electrode having on the front surface of a mica sheet discrete mutually isolated elements or particles of silver photosensitized by exposure to an alkali metal vapor such as caesium vapor the best results are obtained when the tube is treated during exhaust to render the surface conductivity and resultant leakage between particles very low. It has been found that notwithstanding such treatment during exhaust, a certain amount of residual electrical leakage takes place between the photosensitive particles thereby limiting the resolving power of the device, and that further treatment to reduce this electrical leakage makes the photosensitivity of the silver particles considerably less than the maximum obtainable.

The principal object of my invention is to provide an improved cathode ray tube having a mosaic type target electrode of greater photosensitivity and with less electrical leakage between the particles than a conventional type electrode. It is another object to provide an improved and highly sensitized electrode having greater photosensitivity and resolving power than has heretofore been obtainable. It is a further object of my invention to provide a method whereby the photosensitivity and resolving power of a mosaic electrode may be controlled during manufacture.

In accordance with my invention the target electrode having a multiplicity of mutually separated metallic particles is photosensitized in the usual way, such as by exposing the electrode supporting the particles to the vapor of an alkali metal such as caesium and subsequently oxidizing or wholly eliminating the metallic caesium which is deposited between the photosensitive particles. This step of eliminating the metal between the particles is preferably performed while the tube is in normal operation. Further in accordance with my invention the electrode from which the free caesium has been removed between the particles is subsequently baked to increase the photosensitivity of the particles.

Other objects, features and advantages of my invention will appear from the following description taken in connection with the accompanying drawing in which:

Figure 1 is a diagrammatic view illustrating

one form of a television device made in accordance with my invention,

Figure 2 is an enlarged fragmentary sectional view of the photosensitive mosaic electrode during the process of formation and,

Figure 3 is an enlarged fragmentary sectional view made in accordance with my improved method.

A tube made in accordance with my invention is shown in Figure 1 and comprises a highly evacuated glass envelope or bulb 1 with a tubular arm or neck section enclosing a conventional type electron gun and a cylindrical section enclosing a flat target or mosaic electrode 2 so positioned that its front surface may be scanned by a beam of electrons from the electron gun and also may have projected upon it the optical image to be transmitted. Since the image is produced from an object situated outside the tube, that portion or window 3 of the envelope opposite the electrode 2 is made optically uniform so that the image to be transmitted may be projected upon the electrode with a minimum of distortion by the lens system 4.

The electron gun assembly is of the conventional type, and comprises a cathode 5 from which an electron stream may be drawn, a control electrode 6 connected to the usual biasing battery, and a first anode 7 maintained positive with respect to the cathode 5 by a battery 8. The electron stream leaving the first anode 7 is accelerated and concentrated into an electron scanning beam focused on the front surface of the mosaic electrode 2 by a second anode 9, which is preferably a conductive coating on the surface of the bulb 1 extending into the neck of the bulb but removed from that portion through which is projected the optical image to be transmitted. Conventional deflection means, such as deflection coils 10 and 11 may be used to sweep the beam in a horizontal and vertical plane, respectively, to scan the target. It is obvious that conventional electrostatic deflection plates may be substituted for one or both of the deflection coils if desired. The electrode 2 is connected through the impedance 12 to ground and to the collector electrode or second anode 9, and in operation the current flow in this circuit produces a voltage drop across the impedance 12 which may be impressed on the input of a translating device 13, further amplified and applied to a transmitting network in a manner well known to the art.

The mosaic electrode as best shown in Figure 2 comprises an insulating foundation sheet or

base 14, such as a sheet of mica coated with a metal film 15 or other electrically conducting material such as a film of platinum, which serves as a signal electrode from which the picture signals may be obtained. The other side of the sheet of mica has on its surface a plurality of mutually isolated metallic particles 16.

In accordance with my invention the metal particles are photosensitized during the evacuating process of the tube in which the electrode is used by oxidizing the metal particles and subjecting the electrode and oxidized particles to the vapor of an alkali metal such as caesium which deposits not only on the metal particles 16 but also upon the base 14 between the particles which metal between the particles is converted into an electrically non-conducting medium by subjecting the electrode assembly to a controlled quantity of dry oxygen which reacts with the free alkali metal on the base between the particles to form an electrically non-conducting material.

In making the mosaic electrode 2, I select a sheet of mica or other good insulating material having a thickness of approximately .002" and an area sufficient to satisfy the operating requirements of the device in which the electrode is to be used. One surface of the mica sheet is dusted with a finely divided metal compound, such as silver oxide, and the dusted sheet is rapidly heated in an oven at 800° C. until the silver oxide is reduced to silver of which individual and minute portions are drawn up by surface tension to form a multiplicity of microscopic particles 16 spaced from each other, the number and average size of the particles in a unit area being sufficient to satisfy the operating requirements in the way of detail of picture reproduction.

The mosaic surface may be formed, however, in a variety of ways, thus for example, instead of using the metal compound which is applied to the mica base and subsequently reduced and drawn up by surface tension into individual particles, a thin continuous film of silver may be deposited on the base, which film is then broken up into microscopic particles by suitable heat treatment.

The mica sheet or base 14 carrying the silver particles 16 is then mounted in the tube, as shown in Figure 1, the tube evacuated and the silver particles oxidized by admitting oxygen to the envelope to form an oxide coating 17 on each of the silver particles. The excess oxygen is removed from the bulb and the oxidized particles are photosensitized by exposing them to vapor of an alkali metal such as caesium. A conventional way of performing the sensitizing step is to provide a source of caesium, such as a reducible compound of caesium 18 in the annulus 19, which annulus following the photosensitizing step is sealed off and removed from the bulb 1 at the point 20.

During the exposure of the particles to caesium vapor some of the caesium condenses on the surface of the mica base as a metallic film 21 which covers both the oxidized particles 16 and the base 14 between the particles thereby forming an electrical leakage path between the particles and consequently reducing the electrical resistance from particle to particle. A portion of this caesium film 21 which is between the particles may be removed during the evacuating process. However, if sufficient caesium is deposited on the particles to provide optimum pho-

tosensitization, the residual caesium between the particles is sufficient to considerably reduce the insulation between the particles. Following the deposition of caesium, the tube is baked and simultaneously pumped until maximum photosensitivity is obtained and during this baking and pumping some of the free caesium previously condensed as the film 21 on the mica base between the particles is removed. The baking is discontinued when the photosensitivity has increased to a maximum and has decreased very slightly at which point the leakage between the particles due to the presence of caesium between the particles may be still too excessive to satisfy the operating requirements of the device.

In accordance with my invention, the electrodes of the tube are connected, as shown in Figure 1, an optical image of an object projected on the mosaic electrode 2, and the mosaic electrode scanned with the cathode ray beam. The picture signals derived from the signal electrode 15 are amplified by a series of amplifiers, such as the amplifier 13, and the optical image projected on the mosaic electrode 2 is recreated on a viewing tube (not shown). The resolution of the recreated image, which may be defined as the ability to distinguish two lines of an image which are close together, is noted. Oxygen is then liberated within the tube and in the presence of the mosaic electrode, the liberation of oxygen being continued until the resolving power of the mosaic electrode which determines the resolution of the recreated image has passed through a maximum. This indicates that the insulation between the particles has become greater, the metal film 21 being converted into an electrically non-conducting material such as the oxide of the metal. At the same time the operating photosensitivity of the device likewise increases. Care should be taken that just sufficient oxygen is liberated to bring the resolution and the photosensitivity to a maximum as it has been found that following the point at which maximum photosensitivity is obtained, the photosensitivity rapidly decreases with the admission of additional oxygen. Care should likewise be taken that the oxygen is dry as it has been found that if any moisture is present the photosensitization will be decreased.

I prefer to provide a source of oxygen within the tube capable of liberating oxygen in the amount required. For this purpose I provide a source of oxygen such as the nickel filament 22 which contains absorbed oxygen and which is located on the inside wall of the bulb 1 to the rear of the mosaic electrode. I have found that a nickel ribbon filament having a length of 1.5", a width of 0.020", and a thickness of 0.005", coiled to a diameter of 0.25", which has been heated to a temperature of about 900° C. and cooled in an oxygen atmosphere equivalent to 1 mm. of mercury, provides a sufficient source of oxygen for a mosaic electrode having an area of approximately 20 square inches. The nickel filament is supported on the inner wall of the envelope as shown in Figure 1 and while the tube is being operated is gradually heated, such as by current from the battery 23, to drive off oxygen which combines with the caesium on the mica base between the particles. This caesium is converted to caesium oxide which is a relatively poor electrical conductor. The caesium film 21 shown in Figure 2 is thus converted into a film of non-conducting material such as the caesium oxide film 24 shown in Figure 3.

- Following the liberation of oxygen to the proper amount, as indicated by the operation of the device, the photosensitivity of the mosaic electrode is higher than that which is observed prior to the liberation of the oxygen, but may be subsequently increased to a still higher value by baking the tube at a temperature of 200° C. for approximately 7 to 10 minutes or until maximum photosensitivity is obtained.
- 10 Television transmitting tubes when made in accordance with my invention have shown higher sensitivities to light and higher resolution than tubes not made in accordance with my new and improved method. Tubes made in the manner disclosed are more uniform with respect to photosensitivity and resolving power and it has been found that tubes low in photosensitivity and resolving power may be improved considerably by following the teachings of my invention.
- 15 While I do not wish to be limited by any particular theory to explain the improved sensitivity and increased resolution of a television device made in accordance with my invention, it seems probable that the oxygen which is liberated within the tube first reacts with the metallic caesium between the photosensitized metal particles, oxidizing this caesium to caesium oxide which is a relatively poor electrical conductor. It is also believed that the oxygen reacts with part of the free caesium present on the oxidized silver particles, thereby increasing the photosensitivity. During the subsequent baking operation it is believed that free caesium which has been adsorbed by the oxidized silver particles is driven to the surface of the particles, but that this caesium does not migrate to the intervening areas of the base member because the resolution following the baking step is as high as or higher than the resolution prior to baking.
- 20 While I have indicated the preferred embodiments of my invention of which I am now aware and have also indicated only one specific application for which my invention may be employed, it will be apparent that my invention is by no means limited to the exact forms illustrated or the use indicated, but that many variations may be made

in the particular structure used and the purpose for which it is employed without departing from the scope of my invention as set forth in the appended claims.

I claim:

1. The method of photosensitizing a mosaic electrode having a plurality of mutually separated metallic particles on an insulating base supported within a cathode ray tube wherein a cathode ray beam for scanning is developed, which comprises depositing a film of alkali metal on said metallic particles and said base, thermally removing a portion of the alkali metal from areas of the base intermediate the particles, projecting an optical image on said mosaic electrode, tracing the developed cathode ray beam across the said particles to produce signals representative of the surface condition of said electrode, liberating oxygen within said envelope and limiting the amount of liberated oxygen to the point of maximum photosensitivity and resolving power of the mosaic electrode in accordance with observations of the signals resulting from said scanning. 10
- 15 2. The method of photosensitizing a mosaic electrode having a plurality of mutually separated metallic particles on an insulating base supported within a cathode ray tube wherein a cathode ray beam for scanning is developed, which comprises depositing a film of caesium on said metallic particles and said base, thermally removing a portion of the caesium from areas of the base intermediate the particles, projecting an optical image on said mosaic electrode, tracing the developed cathode ray beam across the said particles to produce signals representative of the surface condition of said electrode, liberating oxygen within said envelope and limiting the amount of liberated oxygen to the point of maximum photosensitivity and resolving power of the mosaic electrode in accordance with observations 20 of the signals resulting from said scanning, 25 and subsequently heating the mosaic electrode to a temperature of approximately 200 C. for a predetermined period of time to photosensitize said metallic particles. 30
- 35 40 45

WILLARD HICKOK.